

J. SAVELSBERG.

PROCESS FOR SINTERING SMELTING PRODUCTS AND THE LIKE.

APPLICATION FILED OCT. 21, 1912.

1,103,318.

Patented July 14, 1914.



Witnesses

B. Pommers  
E. Leckert

Inventor  
Josef Savelberg  
by Henry Orth Jr.  
atty

# UNITED STATES PATENT OFFICE.

JOSEF SAVELSBERG, OF PAPENBURG-ON-THE-EMS, GERMANY.

## PROCESS FOR SINTERING SMELTING PRODUCTS AND THE LIKE.

1,103,318.

Specification of Letters Patent. Patented July 14, 1914.

Application filed October 21, 1912. Serial No. 726,942.

*To all whom it may concern:*

Be it known that I, JOSEF SAVELSBERG, a subject of the King of Prussia, residing at 11 Bethlehemkanal, rechts, Papenburg-on-the-Ems, Germany, have invented certain new and useful Improvements in and Relating to the Processes for Sintering Smelting Products and the like; and I do hereby declare the following to be a full, clear, and 10 exact description of the invention.

The present invention relates to improvements for sintering smelting-products and similar materials especially fine granular ores, purple ores and flue dust such fine materials being generally termed fines.

Up to the present time a drawback was experienced in sintering finely divided, granular smelting products for instance fine granular ores, purple ores and flue dust after the ore-briquetting method, as far as the sintering was only very slowly worked in treating many kinds of ores and flue-dust being mixed with fuel, because the products to be sintered in their upper portion about 25 five or six inches from the surface of the charge are maintained partially suspended by and in the air current and thereby do not remain in sufficient contact with the fuel of the mixture to be sintered. In order to 30 prevent such separation of said ore-material and fuel the moistening of the mixed materials in the most ores is not feasible in respect to many materials, as the latter, for instance some kinds of purple ores and flue 35 dust will only be moistened with much difficulty or not at all.

The present invention avoids all these inconveniences by adding steam to the air forced through the materials to be sintered. 40 If these ore-materials are too fine or too dust-like for being handled without injuring health the same must be sprayed with water—as is necessary according to the laws of at least several countries—before being 45 charged into the treating vessel or furnace. This steam being employed in a suitably

sufficient proportion is condensed in the colder layers, consequently also in the upper layers of the materials to be sintered, so that a superficial moistening of the upper 50 layers of the materials to be sintered will take place and thus prevent a separation of the material to be sintered from the parts of fuel. Part of the steam is also decomposed by the glowing (incandescent) parts 55 of the fuel, so that the water gas formed will favorably promote at the same time by its presence and high temperature of combustion the sintering and a further portion of the steam escapes as primed steam from the 60 sintering receptacle or furnace, and is clearly visible as a cloud of highly primed steam issuing from the cover of the furnace.

In the drawing, showing a suitable form of furnace, A is a cover connected to a suitable outlet flue *a* serving to conduct the generator gas and excess steam from the furnace. This cover rests on a shallow sintering chamber or converter C, mounted by means of trunnions B on a suitable carriage 70 K. This converter has a grate, or perforated bottom R beneath which air is admitted through pipe L and the steam through pipe D.

I claim:

The process of sintering non-sulfurous ore fines and flue dust, which comprises mixing the material with carbonaceous material and blowing the same with air and excess of steam sufficient to form water gas by combining with the carbonaceous material and to condense in the upper portion of the charge and wet the same to prevent it from being blown away by the force of the blast.

In testimony whereof I have signed my 85 name to this specification in the presence of two subscribing witnesses.

JOSEF SAVELSBERG.

Witnesses:

JEAN GRUND,  
CARL GRUND.